

## UNITED STATES PATENT OFFICE

2,285,452

## LUBRICATING COMPOUND

George E. Merkle, Glen Ridge, N. J., assignor to  
 Lubriplate Corporation, New York, N. Y., a  
 corporation of New York

No Drawing. Application February 26, 1940,  
 Serial No. 320,894

2 Claims. (Cl. 252—18)

The invention relates to a lubricant of the same or similar type as that of U. S. Patent No. 2,043,638, wherein it was disclosed that finely divided zinc oxide dispersed in an oily lubricating medium improves the lubricating qualities of that medium. This invention is based on the discovery that basic lead carbonate similarly dispersed in oily bases, and under proper amount and conditions, will likewise produce lubricants of better lubricating value than the base itself, forming new lubricating compositions having uses in many directions.

The conditions under which this material operates with the effect stated require that it be sufficiently finely divided, to retain its dispersed condition, and in this respect, the finer grades of basic carbonate to be had on the market are sufficiently fine, also that the oily components in which it is dispersed be of such character or so combined as not to saponify the carbonate, and finally, that the carbonate be present in amount not less than 3½% nor more than 15%.

Departing in either direction from the percentage range just stated produces negative or opposite effects, which is to say, results in more rapid wear of the bearing surfaces than would occur by the use of the base alone, without the carbonate. Within the limits the reduction in the rate of wear, as compared to the base without the addition, is substantial; for example, where a given oily base resulted in bearing wear to the extent of 3.75 units, a composition of the same base with 5% of basic lead carbonate dispersed in it and unsaponified, tested under precisely identical conditions, produced only 2.5 units of wear, indicating an improvement in the order of 33%. Some variation may be expected as between different bases, but consistently good results are obtained by the use of about 5%. With most bases even a slight increase above the range results in wear equal to that of the base alone or no improvement while further increase results in serious abrasion.

As examples, the following formulae are given:

Per cent 45

|                                                                                            |       |
|--------------------------------------------------------------------------------------------|-------|
| (1) Animal or vegetable fats saponified<br>with $\text{Ca}(\text{OH})_2$ to a neutral soap | 10-12 |
| Refined neutral mineral oils of from<br>300-500 Saybolt at 100° F                          | 85-83 |
| Basic lead carbonate                                                                       | 5 50  |
| (2) Cylinder stock                                                                         | 85    |
| Lead naphthenate                                                                           | 10    |
| Basic lead carbonate                                                                       | 5     |

In both cases the components are thoroughly mixed at a temperature not higher than 180° F., any ordinary mill or agitator being sufficient. In all cases the oily and any other materials used are selected or neutralized so as to have no saponifying action on the carbonate and so that the latter remains present in a free state and within the limits stated.

It will be understood that the base is compounded with reference to the general characteristics required of the final product and is subject to variation in character or quantity, according to the practice in the art, to adapt the lubricant to the nature of the work. The amount of carbonate requisite to produce the effect above referred to is also sufficient to impart to the lubricant a strong white color persisting even after long-continued use; which is to say, it does not turn black with wear, making it especially desirable from the point of cleanliness. Such lubricant has the quality of producing a highly polished surface on the bearing faces of ordinary journals which is similar to that of the above mentioned patent and continues permanently with a noticeable reduction in the rate of wear.

I claim:

1. A lubricant of the class consisting of oil and grease bases, said lubricant having a base which constitutes at least 85% of the lubricant and contains finely divided, unsaponified, basic lead carbonate dispersed therein to the extent of not less than 3½% nor more than 15% by weight.

2. A lubricant of the class consisting of oil and grease bases, said lubricant having a base which constitutes approximately 95% of the lubricant and is free of saponifying agent and contains dispersed therein finely divided basic lead carbonate in the amount of approximately 5% by weight of the lubricant.

GEORGE E. MERKLE.